

# United States Patent Office

3,033,674

Patented May 8, 1962

1

3,033,674

**SMEILING OF ZINC IN CERAMIC RETORTS**  
 Kenneth A. Phillips, Collingsville, Ill., assignor to American Zinc, Lead and Smelting Company, St. Louis, Mo., a corporation of Maine  
 No Drawing. Filed Dec. 16, 1959, Ser. No. 859,862  
 1 Claim. (Cl. 75—86)

This invention relates to the smelting of zinc. One process by which zinc metal is commonly produced involves mixing zinc oxide, which may be in the form of zinc sinter, with carbonaceous reducing material and sodium chloride, charging banks of "horizontal" retorts with the mixture, heating the retorts externally, and condensing the reduced zinc metal. The retorts are commonly hollow cylinders of ceramic material, oriented transversely of a long furnace, with their inner ends supported on a longitudinal center wall and with their mouths opening through a side wall of the furnace, much like boiler tubes in a header. The retorts are arranged in banks symmetrically about the center wall, so that two chambers full of retorts are provided, one on either side of the center wall, the retorts opening through opposite long side walls of the furnace. The retorts are heated, externally, by hot gases in the space between the center wall and the side wall through which the retorts open. The retorts, which are about ten inches in (outside) diameter, and five feet long, must be substantially impervious to zinc vapor, resistant to attack by coal ash and the gangue constituents of zinc ore, must have high strength and good resistance to plastic flow at temperatures up to about 2300° F. They must be transferred, at high heat, from the firing kiln or a soaking pit, to the furnace; a retort whose temperature after firing drops below 1600° F. being almost certain to fail quickly. Industry wide, the average life of silica retorts is about 45 days. It can be seen, then, that it is of the utmost importance that the deterioration of the retorts, which is rapid enough as it is, be not accelerated.

Immediately outside the side walls of the furnace, the open ends of the retorts are capped with condensers, which are in the form of truncated cones. The ends of these cones are "stuffed" with wet anthracite or coke, in such a way that the carbon monoxide produced in the reaction between the carbonaceous material and the zinc oxide, can escape, and that most of the metal fumes cannot. The condensers are maintained at a heat sufficiently high to keep the zinc molten, but low enough to condense the metal vapors. For example, the retorts may be kept at about 2150° F. and the condensers at about 950° F. From time to time, the plug in the condensers is knocked out, and the zinc metal is tapped.

As has been indicated above, sodium chloride, common salt, is used in the charging mixture. Without the use of this salt or other suitable chloride, the recovery of zinc metal is relatively low, because of the formation of what is known as blue powder, fine particles of zinc metal coated with a substantially monomolecular layer of zinc oxide. This metal is not lost in the process, but simply recirculates, lowering the efficiency of the process. When sodium chloride or zinc chloride is used, the condenser surface is coated with a flux, which encourages the wetting of the surface by the zinc metal, and permits the recovery in a single cycle of about 85% of the zinc vapor as molten zinc. In a high-lead zinc ore, the presence of the lead facilitates the condensing of the zinc. When a low-lead zinc is desired, a zinc ore low in lead must be used, and the recovery of the zinc in liquid form is more difficult, and the use of an efficient halide flux is doubly important.

It was suggested in an early patent (Moulden et al., No. 1,030,676) that other halides might be used as

2

"fluxes" in the reduction process, but chlorides are the only specific examples given. It has been known in soldering fluxes, to use a mixture of chlorides and fluorides. It has also been known to use a mixture of chlorides and fluorides in the recovery of zinc metal from dross, cf. Lytle, No. 2,578,977 and Deterding, No. 2,701,194. The addition of fluorides has been known to tend to make the contaminated metal easier to coalesce into a liquid pool. However, in the primary smelting process, the use of even one percent of fluorite by weight of sinter results in a very serious attack on the refractory walls of the retorts. The degree of attack is roughly proportional to the percentage of fluorite added. Although the evidence is somewhat difficult to evaluate, it is believed that the degree of attack is also increased when coarse particles of fluorite are employed.

One of the objects of this invention is to provide a more efficient method of smelting zinc ores in ceramic retorts, which utilizes the fluxing capacity of fluorides without seriously damaging the retorts.

Other objects will become apparent to those skilled in the art in the light of the following description.

In accordance with this invention, generally stated, a process of smelting zinc ores in refractory retorts is provided, in which a relatively small amount of finely-ground fluorite is used in conjunction with sodium chloride, in such a way as to unexpectedly increase the recovery of metallic zinc over the recovery to be expected from the use of either the fluorite or the salt, singly. The process of this invention does not lead to uneconomic deterioration of the retorts.

The fineness to which the fluorite is ground seems to determine its effectiveness as a fluxing medium, its efficiency varying, within limits, inversely as the particle size. However, merely using finely-ground fluorite alone does not give the desired results. In order to achieve the desired fluxing, it is necessary that the fluorite be admixed with common salt in the charge mix.

An example of the process of this invention, and a comparison of the results obtained with it, and the results obtained by conventional methods, and results obtained with the use of fluorite alone, is as follows:

### Example 1

Retorts approximately 9 1/4 inches in diameter and 61 inches long, inside dimensions, were filled with thoroughly mixed charges having the compositions shown below.

|                            | Dry pounds of material charged |          |          |
|----------------------------|--------------------------------|----------|----------|
|                            | Retort 1                       | Retort 2 | Retort 3 |
| Sinter, 65% Zn             | 180                            | 180      | 180      |
| Reduction fuel, 86% C      | 55                             | 55       | 55       |
| Salt, NaCl                 | 3                              | 0        | 3        |
| Fluorite, CaF <sub>2</sub> | 0                              | 2        | .36      |

The charge of retort 1 represents a conventional charge. The charge of retort 2 represents a simple substitution of fluorite for common salt. In retort 2, the fluorite was ground moderately fine, with 85% of it passing a 200 mesh screen. Retort 3 represents the charge used in the process of this invention. The fluorite in retort 3 was ground sufficiently fine so that all of it passed a 200 mesh screen.

The temperature of the gases surrounding the retorts at the beginning of the forty-eight hour cycle was 1750° F.; the temperature at the conclusion of the cycle was 2220° F. The zinc metal was drawn four times during the cycle. The fumes leaving the condensers were burned, cooled and filtered to recover the solid contents thereof. The

following data represent the averages for a number of retorts charged and treated in the same way.

|                      | Dry pounds of product |     |     | Pounds of zinc contents |       |       |
|----------------------|-----------------------|-----|-----|-------------------------|-------|-------|
|                      | 1                     | 2   | 3   | 1                       | 2     | 3     |
| Sinter charged.....  | 180                   | 180 | 180 | 117.0                   | 117.0 | 117.0 |
| Slab zinc drawn..... | 84                    | 88  | 86  | 83.5                    | 82.8  | 86.1  |
| Ladle skimmings..... | 14                    | 15  | 13  | 9.1                     | 9.8   | 7.8   |
| Rich residues.....   | 46                    | 46  | 45  | 16.1                    | 16.1  | 14.9  |
| Lean residues.....   | 50                    | 50  | 50  | 2.5                     | 2.5   | 2.5   |
| Condenser fume.....  | 5                     | 5   | 5   | 3.8                     | 3.8   | 3.8   |

The ladle skimmings are drawn from the condenser, along with the liquid metal therein. They contain the coal or coke used to stuff the condenser and all zinc particles or zinc compounds which are not collected as liquid metal and cast into slabs. The ladle skimmings and rich residues from the front of the retort are recirculated in the next mixed charge. The lean residues are discarded or are treated by some method other than retort smelting. In commercial operations the condenser fume is not collected; it is wasted to the atmosphere.

The simultaneous use in retort 3 of 1.67% of salt and 0.20% of fluorite, based upon the sinter weight, raised the output of slab zinc by over 3%. In retorts 1 and 2 the use of one halide alone allowed an equivalent amount of zinc to partially oxidize and to enter the blue powder. The latter is recirculated on the following charge, and most of the zinc is recovered in the second pass through the furnace, but the retreatment step reduces furnace capacity and increases operating costs.

It should be noted that the large amount of fluorspar in the charge of retort 2 had a seriously deleterious effect upon the ceramic surface of the retort, whereas the small amount of fine fluorspar of the charge in retort 3 had no discernible deleterious effect upon the retort.

#### Example 2

Retorts approximately 9 1/4 inches in diameter and 61 inches long, inside dimensions, were filled with thoroughly mixed charges having the compositions shown below. The fluorite in retort 1 was ground very finely, so that all of it would pass a 200 mesh screen. The fluorite in retort 2 was ground only to pass through a 10 mesh screen.

|                                  | Dry pounds of material charged |          |
|----------------------------------|--------------------------------|----------|
|                                  | Retort 1                       | Retort 2 |
| Sinter, 65% Zn.....              | 180                            | 180      |
| Reduction fuel, 86% C.....       | 55                             | 55       |
| Salt, NaCl.....                  | 3                              | 3        |
| Fluorite, CaF <sub>2</sub> ..... | .36                            | 1.08     |

The temperature of the gases surrounding the retorts at the beginning of the 48-hour cycle was 1750° F.; the temperature at the conclusion of the cycle was 2220° F. The zinc metal produced was drawn four times during the cycle. The fumes leaving the condensers were burned, cooled and filtered to recover the solid contents thereof. Pertinent data are tabulated below. Each column of figures shows the averages for a number of retorts charged and treated in the same way.

|                      | Dry pounds of product |          | Pounds of zinc contents |          |
|----------------------|-----------------------|----------|-------------------------|----------|
|                      | Retort 1              | Retort 2 | Retort 1                | Retort 2 |
| Sinter charged.....  | 180                   | 180      | 117.0                   | 117.0    |
| Slab zinc drawn..... | 86                    | 86       | 86.0                    | 86.1     |
| Ladle skimmings..... | 13                    | 13       | 7.8                     | 7.7      |
| Rich residues.....   | 45                    | 45       | 14.9                    | 14.8     |
| Lean residues.....   | 50                    | 50       | 2.5                     | 2.5      |
| Condenser fume.....  | 5                     | 5        | 3.8                     | 3.9      |

The table above shows that 0.36 lb. of fine fluorite was as effective in promoting the condensation of zinc as was 1.08 lbs. of coarse fluorite. To be effective, the fluorine in the fluorite must be carried to the condenser, where it will enter a chloride-fluoride flux. The following table shows that substantially equal amounts of fluorine travel to the condenser when a small amount of fine fluorite is used as when a larger amount of coarse fluorite is used.

| 5                    | 10 | Assay percent fluorine in products |         |          |         |
|----------------------|----|------------------------------------|---------|----------|---------|
|                      |    | Retort 1                           |         | Retort 2 |         |
|                      |    | Trial 1                            | Trial 2 | Trial 1  | Trial 2 |
| Ladle skimmings..... |    | .25                                | .28     | .24      | .26     |
| Condenser fume:      |    |                                    |         |          |         |
| Before 1st draw..... |    | .18                                | .13     | .20      | .15     |
| 1st to 2nd draw..... |    | .08                                | .09     | .09      | .19     |
| 2nd to 3rd draw..... |    | .11                                | .17     | .14      | .14     |
| 3rd to 4th draw..... |    | .15                                | .22     | .20      | .13     |
| Averages.....        |    | .13                                | .15     | .16      | .15     |

The metallurgical results were therefore alike; the physical results are different. The small amount of fluorite used in the retorts marked "1" did not seriously damage the retorts used; the larger amount of coarse fluorite used attacked the retorts marked "2" seriously enough to render the use of fluorite uneconomic at some smelters.

#### Example 3

30 Retorts approximately 9 1/4 inches in diameter and 61 inches long, inside dimensions, were filled with thoroughly mixed charges having the compositions shown below. The fluorite in retort 1 was ground very finely, so that all of it would pass a 200 mesh screen. The fluorite in retort 2 was ground only through a 10 mesh screen.

|                                  | Dry Pounds of Material Charged |          |
|----------------------------------|--------------------------------|----------|
|                                  | Retort 1                       | Retort 2 |
| Sinter, 65% Zn.....              | 180                            | 180      |
| Reduction fuel, 86% C.....       | 55                             | 55       |
| Salt, NaCl.....                  | 3                              | 3        |
| Fluorite, CaF <sub>2</sub> ..... | .12                            | .36      |

40 The temperature of the gases surrounding the retorts at the beginning of the 48-hour cycle was 1750° F.; the temperature at the conclusion of the cycle was 2220° F. The zinc metal produced was drawn four times during the cycle. The fumes leaving the condensers were burned, cooled and filtered to recover the solid contents thereof. Pertinent data are tabulated below. Each column of figures shows the averages for a number of retorts charged and treated in the same way.

| 50                   | 60 | Dry pounds of product |          | Pounds of zinc contents |          |
|----------------------|----|-----------------------|----------|-------------------------|----------|
|                      |    | Retort 1              |          | Retort 2                |          |
|                      |    | Retort 1              | Retort 2 | Retort 1                | Retort 2 |
| Sinter charged.....  |    | 180                   | 180      | 117.0                   | 117.0    |
| Slab zinc drawn..... |    | 84                    | 84       | 83.5                    | 83.7     |
| Ladle skimmings..... |    | 14                    | 14       | 9.0                     | 9.2      |
| Rich residues.....   |    | 46                    | 45       | 15.7                    | 15.3     |
| Lean residues.....   |    | 50                    | 51       | 2.5                     | 2.5      |
| Condenser fume.....  |    | 5                     | 5        | 3.8                     | 3.8      |

65 This series of tests showed that the beneficial effects of fluorite substantially disappeared when the amount of fine fluorite used was decreased below 0.1% of the sinter weight or when the amount of coarse fluorite used was decreased below 0.3% of the sinter weight. Within the practical limits of testing retort performance, retorts 1 and 2 of Example 3 gave the same results as retort 1 in Exam-

ple 1. No significant attack of the fluorite was noted upon the retorts used in the series of tests covered by Example 3.

It is therefore believed that the amount of fluorite added should not be less than 0.1% nor more than 0.6% of the sinter weight. The best balance between recovery and retort life is achieved when 0.2% to 0.3% of finely-ground fluorite is used, with about 0.5 to 2.0% of common salt, by weight of the sinter. At least 90% of the fluorite should pass a 150 mesh screen.

Having thus described the invention, what is claimed and desired to be secured by Letters Patent is:

The method of smelting zinc ore in ceramic retorts comprising charging said retorts with a mixture of oxidic zinc ore, reduction fuel, sodium chloride and fluorite, at least 90% of the fluorite being of a fineness at least to pass a 150 mesh screen, said sodium chloride being present in the charging mixture in an amount between about 0.5 and 2.0 percent by weight of the oxidic zinc ore and the said fluorite being present in the charging mixture in an amount between about 0.1 and 0.6 percent by weight of the oxidic zinc ore, heating said retorts and said mixture to a temperature at which, over a period of time, the major portion of the oxidic zinc ore is reduced to metallic zinc

and converted to zinc vapor, and condensing said zinc vapor.

References Cited in the file of this patent

UNITED STATES PATENTS

|    |           |           |               |
|----|-----------|-----------|---------------|
| 5  | 79,701    | Stevens   | July 7, 1868  |
|    | 713,043   | Armstrong | Nov. 4, 1902  |
|    | 1,999,209 | Queneau   | Apr. 30, 1935 |
| 10 | 2,578,977 | Lytle     | Dec. 18, 1951 |
|    | 2,701,194 | Deterding | Feb. 1, 1955  |
|    | 2,867,037 | Lawton    | Jan. 6, 1959  |

OTHER REFERENCES

- 15 Hackh's Chemical Dictionary, by Julius Grant, 3rd Edition, The Blakiston Co., 1944, page 214 relied upon.  
 Chambers' Technical Dictionary, by C. F. Tweney and L. E. C. Hughes, Revised Edition with Supplement, 1944, the Macmillan Co., page 177 relied upon.
- 20 Chemical Encyclopedia, by C. T. Kingzett, 3rd Edition, D. Van Nostrand Co., 1924, page 145 relied upon.  
 Chemical Engineers Handbook, by Perry, 3rd Edition, McGraw-Hill Book Co. Inc., 1950, page 1111 relied upon.